

T. YANAI.

COPPER CONDUCTOR FOR ELECTRIC LAMP BULBS AND OTHER VACUUM TUBES,  
APPLICATION FILED MAY 29, 1918.

1,417,287.

Patented May 23, 1922.

*Fig. 1.*



*Fig. 2.*



INVENTOR;

By Teizo Yanai

Mr. Wallace White  
ATTY.

# UNITED STATES PATENT OFFICE.

TEIZO YANAI, OF TOKYO, JAPAN, ASSIGNOR TO NIHON DENKI KOGIJO KABUSHIKI KAISHA, OF TOKYO, JAPAN.

## COPPER CONDUCTOR FOR ELECTRIC-LAMP BULBS AND OTHER VACUUM TUBES.

1,417,287.

Specification of Letters Patent. Patented May 23, 1922.

Application filed May 29, 1918. Serial No. 237,183.

To all whom it may concern:

Be it known that TEIZO YANAI, subject of the Emperor of Japan, residing at No. 6 Shichome, Atagoshita Machi, Shiba Ku, Tokyo, Japan, have invented new and useful Improvements in Copper Conductors for Electric-Lamp Bulbs and Other Vacuum Tubes, of which the following is a specification.

10 This invention relates to leading-in conductors of electric lamp bulbs and the like, which consists of slender copper tubes sealed in glass rods and to a process of forming such conductors. The object of this invention is to obtain a cheap substitute for platinum which is usually employed for the purpose, by the use of a copper conductor which is made hollow, the conductor being thus made somewhat flexible and crevices being prevented from appearing between the conductor and the glass rod in which it is sealed, due to difference of the coefficient of expansion of copper and glass.

15 In the accompanying drawings, Fig. 1 shows a tube formed by winding or bending a long thin skelp of copper, and Fig. 2 shows copper tubes sealed in a glass rod in accordance with this invention.

20 Hitherto there have been incandescent electric lamps and other vacuum tubes with leading-in conductors of copper, but in such bulbs and vacuum tubes, although the surface of the conductors and the glass rods tightly stick together, there is a drawback

25 of their not perfectly maintaining vacuum, crevices being formed, when subjected to changes of temperature between the copper wire and the glass rod due to the difference of coefficients of expansion of the two. The

30 present invention is an improvement on the above, and consists in the use of copper wire which is made hollow, thus a certain degree of flexibility being given thereto and the separation of the wire from the glass being

35 effectively prevented notwithstanding the strain caused between the two when subjected to change of temperature due to differences in their coefficients of expansion.

40 The following is an example of one man-

ner in which my invention may be put into practice:—

Take a thin copper wire and press part of it flat and thin by a roller or any other suitable means. Bend this flattened part into a tube, joining the edge (1) with the edge (2), as shown in Fig. 1, and leaving vacant place (3) within. A conducting wire 6 formed of any suitable material is now inserted into the tubular portion, whereupon the front end 5 thereof is pressed toward the wire 6 so that the tubular portion is closed. The tube and wire are now inserted into the glass wall of the bulb, whereupon the glass is subsequently heated to a semi-melted condition. The heating is continued for a while and the glass rod is pressed flat as far as the hollowness of the copper tube is not interfered with. Thus the copper tube is hermetically sealed, and a glass rod with hollow space within, which hollow space being surrounded by copper, is formed.

I am aware that before this invention there is known a leading-in wire of metal tube used with vacuum containers such as vapor lamps or vapor rectifiers through which a large amount of electric current passes; but such leading-in wire cannot practically be used with ordinary incandescent lamp bulbs. Now, according to my invention, a copper tube is formed by bending one edge of a thin narrow strip of that metal over the other edge, and a very slender tube can very easily be formed by simply passing a very narrow thin strip through a die.

I claim:

85 A leading-in conductor for vacuum containers comprising a single length of material having a slit tube formed integral therewith at one end thereof, the longitudinal edges of said tube overlapping, and a wire closing the open end of the tube.

In testimony whereof I have signed my name to this specification in the presence of two subscribing witnesses.

TEIZO YANAI.

Witnesses:

H. F. ALTMANS,  
YOSHIO KAWADA.